# EUROPEAN PATENT SPECIFICATION

(11) **EP 3 730 655 B1**
(45) Date of publication and mention of the grant of the patent: **18.05.2022**
(21) Application number: 18891912.0
(22) Date of filing: 28.11.2018
(51) Int. Cl.: C22C 38/42, C22C 38/44, C22C 38/46, C22C 38/48, C22C 38/00, C22C 38/50, C21D 8/02, C21D 9/46, C21D 1/18, C22C 38/02, C22C 38/04, C22C 38/06

(54) **HIGH STRENGTH STEEL PLATE AND MANUFACTURING METHOD THEREFOR**
HOCHFESTE STAHLPLATTE UND HERSTELLUNGSVERFAHREN DAFÜR
PLAQUE D'ACIER À HAUTE RÉSISTANCE ET SON PROCÉDÉ DE FABRICATION

(30) Priority: 24.12.2017 KR 20170178924
(43) Date of publication of application: 28.10.2020
(73) Proprietor: POSCO, Gyeongsangbuk-do 37859 (KR)
(72) Inventor: HONG, Soon-Taik, Pohang-si, Gyeongsangbuk-do 37877 (KR)
(74) Representative: Potter Clarkson
(86) International application number: PCT/KR2018/014855
(87) International publication number: WO 2019/124793

(56) References cited:
- WO-A2-2010/074473
- JP-A- 2014 218 707
- JP-A- 2015 124 435
- JP-A- 2015 124 435
- KR-A- 20100 076 745
- KR-A- 20110 061 260
- KR-A- 20150 101 735
- KR-A- 20150 126 683
- KR-A- 20160 078 573
- KR-B1- 100 833 069
- KR-B1- 100 833 069

## Description

### [Technical Field]

The present disclosure relates to a high strength steel plate and a manufacturing method therefor, and more particularly, to a high strength steel plate having excellent tensile strength and impact toughness, particularly suitable for a nuclear reactor containment container, and a manufacturing method therefor.

### [Background Art]

Various materials are used for the structures and facilities of a nuclear power plant according to the type, usage, and safety properties thereof. In particular, a nuclear reactor containment vessel utilizes a steel material, and A516-70 steel produced by a normalizing process is mainly used as a thick steel plate material.

However, such A516-70 steel has insufficient tensile strength (about 500 Mpa) to ensure the nuclear power plant's safety, and, thus, a range of use thereof may be extremely limited. That is, since the A516-70 steel has relatively low tensile strength, when used to manufacture a nuclear reactor containment vessel, there may be a risk of damage or explosion due to the failure to withstand the high pressure inside. Accordingly, there may be an urgent need to develop a material suitable for a nuclear reactor containment container while having tensile strength of a certain level or more.

In order to improve the tensile strength, if a relatively large amount of expensive alloying elements is added to a steel material or a separate heat treatment is performed, tensile strength may be hardly improved, but an increase in costs due to the addition of the alloying elements may be inevitable, and there may be other incidental problems involved.

Patent Document 1 discloses a high strength steel plate with improved tensile strength, which may be a high strength steel plate that may be used for a nuclear reactor containment vessel. However, the steel plate disclosed in Patent Document 1 has a level of tensile strength that may be used as a steel plate for a nuclear reactor containment vessel, but may not be suitable as a material for a nuclear reactor containment vessel due to deteriorations in low-temperature toughness and nil-ductility transition temperature properties.

Patent document 2 discloses a high strength steel plate including, by weight: 0.03% to 0.20% C, 0.15% to 0.55% Si, 0.9% to 1.5% Mn, 0.001% to 0.05% Al, 0.030% or less P, 0.030% or less S, 0.30% or less Cr, 0.2% or less Mo, 0.6% or less Ni, 0.07% or less V, 0.04% or less Nb, 5 ppm to 50 ppm Ca, 0.005% to 0.025% Ti, 0.0020% to 0.0060% N, 0.0005% to 0.0020% B, the balance of F and unavoidable impurities. The steel plate may be formed of tempered martensite, and conditions for cooling and recrystallization controlled rolling are optimized so as to control an average grain size of a microstructure and an aspect ratio of structure grains.

Patent Document 3 discloses a thick steel plate for a reactor storage container having a composition comprising, by mass, 0.05 to 0.15% C, 0.05 to 0.60% Si, 0.8 to 1.8% Mn, 0.020% or lower of P, 0.005% or lower of S, 0.005 to 0.080% Al and 0.0005 to 0.0050% N and further comprising one or more kinds selected from 0.50% or lower of Cu, 0.70% or lower of Ni, 0.50% or lower of Cr, 0.40% or lower of Mo, 0.07% or lower of V and 0.0003 to 0 . 0020% B, and in which plate thickness satisfies 100 mm or lower, the microstructure in the 1/4 position of the plate thickness is made of tempered lower bainite and tempered martensite, and Tin an NRL drop hammer test in the 1/4 position of the plate thickness is -55°C or lower.
(Patent Document 1) Korea Patent Publication No. 10-2010-0076745 (published on July 6, 2010)
(Patent Document 2) WO 2010/074473 A2 (published on 1 July 2010)
(Patent Document 3) JP 2015124435 A (published on 6 July 2015)

### [Disclosure]

### [Technical Problem]

According to an aspect of the present disclosure, a high strength steel plate having excellent tensile strength, low-temperature toughness, and nil-ductility transition temperature properties, particularly suitable for a nuclear reactor containment container of a nuclear power plant, and a manufacturing method therefor, may be provided.

### [Technical Solution]

According to an aspect of the invention, a high strength steel plate includes, by weight: 0.05 to 0.20% of C, 0.15 to 0.55% of Si, 0.9 to 1.75% of Mn, 0.001 to 0.05% of Al, 0.03% or less of P, 0.03% or less of S, 0.05 to 0.3% of Cr, 0.05 to 0.6% of Ni, 0.005 to 0.35% of Cu, 0.05 to 0.2% of Mo, 0.005 to 0.07% of V, 0.005 to 0.04% of Nb, 0.0005 to 0.005% of Ca, 0.005 to 0.025% of Ti, 0.002 to 0.006% of N, less than 0.0005% of B, and a balance of Fe, with inevitable impurities, satisfies relationships of Cu + Ni + Cr + Mo: 1.5% or less, Cr + Mo: 0.4% or less, V + Nb: 0.1% or less, and Ca/S: 1.0 or higher, and includes a microstructure of 30 to 60 area% of tempered martensite and 40 to 70 area% of tempered bainite, wherein the sum of the tempered martensite and the tempered bainite is 100 area%, wherein a grain aspect ratio as defined herein of the microstructure is 1.1 to 2.5,
wherein Charpy impact toughness of the steel plate is 300J or more at -60°C, and wherein the low-temperature impact toughness is evaluated as a Charpy impact energy value obtained by performing a Charpy impact test on a specimen having a V notch at -60°C.

The tempered martensite may be included in 40 to 60 area% in the microstructure, and the tempered bainite may be included in 40 to 60 area% in the microstructure.

A nil-ductility transition temperature of the steel plate may be -50°C or lower, wherein the nil-ductility transition temperature is a result value according to the drop-weight test transition temperature set by the ASTM E208-06 method.

Tensile strength of the steel plate is 600 MPa or more.

According to an aspect of the invention, a method of manufacturing a high strength steel plate includes: reheating a steel slab at 1050 to 1250°C, the steel slab comprising, by weight: 0.05 to 0.20% of C, 0.15 to 0.55% of Si, 0.9 to 1.75% of Mn, 0.001 to 0.05% of Al, 0.03% or less of P, 0.03% or less of S, 0.05 to 0.3% of Cr, 0.05 to 0.6% of Ni, 0.005 to 0.35% of Cu, 0.05 to 0.2% of Mo, 0.005 to 0.07% of V, 0.005 to 0.04% of Nb, 0.0005 to 0.005% of Ca, 0.005 to 0.025% of Ti, 0.002 to 0.006% of N, less than 0.0005% of B, and a balance of Fe, with inevitable impurities, satisfying relationships of Cu + Ni + Cr + Mo: 1.5% or less, Cr + Mo: 0.4% or less, V + Nb: 0.1% or less, and Ca/S: 1.0 or higher, rolling the slab in a temperature range of Tnr to Tnr + 100°C, wherein Tnr is determined in accordance with Equation 1 hereof, to provide a steel plate, austenizing the steel plate in a temperature range of 870 to 950°C, quenching the austenized steel plate to a temperature range of 300°C or lower, and tempering the quenched steel plate in a temperature range of 595 to 700°C, wherein a cumulative reduction amount of the rolling is 50 to 90%, and wherein a grain aspect ratio as defined herein of a microstructure of the steel plate by the rolling is controlled to have a range of 1.1 to 2.5, $Tnr \left(°C\right) = 887 - 464 \times C + 890 \times Ti + 363 \times Al - 357 \times Si + \left(\begin{matrix}6445 \times Nb - 644 \times N \\ {b}^{1 / 2}\end{matrix}\right) + \left(732\times V-230\times {V}^{1 / 2}\right) .$

The austenizing may be performed for a time period of 1.6 * t (where, t denotes a thickness (mm) of the steel plate) + (10 to 30 minutes).

The tempering may be performed for a time period of 2.4 * t (where, t denotes a thickness (mm) of the steel plate) + (10 to 30 minutes).

### [Advantageous Effects]

According to an aspect of the present disclosure, a high strength steel plate securing a tensile strength of 600 MPa or more, a Charpy impact toughness of 300 J or more at -60°C, and a nil-ductility transition temperature of -50°C or lower, to be particularly suitable for a nuclear reactor containment container of a nuclear power plant, and a manufacturing method therefor, is provided.

### [Best Mode for Invention]

The present disclosure relates to a high strength steel plate and a manufacturing method therefor, and, hereinafter, preferred embodiments of the present disclosure will be described. Embodiments of the present disclosure may be modified in various forms, and the scope of the present disclosure should not be construed as being limited to embodiments to be described below. These embodiments may be provided to those skilled in the art to further detail the present disclosure.

Hereinafter, the steel composition of the present disclosure will be described in more detail. Hereinafter, unless otherwise indicated, % representing the content of each element is based on weight.

A high strength steel plate according to an embodiment of the present disclosure comprises, by weight: 0.05 to 0.2% of C, 0.15 to 0.55% of Si, 0.9 to 1.75% of Mn, 0.001 to 0.05% of Al, 0.03% or less of P, 0.03% or less of S, 0.05 to 0.3% of Cr, 0.05 to 0.6% of Ni, 0.005 to 0.35% of Cu, 0.05 to 0.2% of Mo, 0.005 to 0.07% of V, 0.005 to 0.04% of Nb, 0.0005 to 0.005% of Ca, 0.005 to 0.025% of Ti, 0.002 to 0.006% of N, less than 0.0005% of B, and a balance of Fe, with inevitable impurities.

Carbon (C): 0.05 to 0.2%

Since carbon (C) may be an effective element for securing strength, the present disclosure limits a lower limit of the carbon (C) content to 0.05% to prevent a decrease in strength on a matrix phase. When carbon (C) is excessively added, toughness and weldability may be deteriorated, making it unsuitable for use for a nuclear reactor containment container, and the present disclosure limits an upper limit of the carbon (C) content to 0.2%. Therefore, the carbon (C) content of the present disclosure is 0.05 to 0.2%, and a preferable carbon (C) content may be 0.08 to 0.15%.

### Silicon (Si): 0.15 to 0.55%

Silicon (Si) may be an element added for a deoxidation effect, a solid solution strengthening effect, and an impact transition temperature increasing effect. Therefore, the present disclosure limits a lower limit of the silicon (Si) content to 0.15% to achieve this effect. A preferred lower limit of the silicon (Si) content may be 0.2%, and a more preferred lower limit of the silicon (Si) content may be 0.3%. When the silicon (Si) is excessively added, weldability of the steel plate may be deteriorated and an oxide film may be severely formed on a surface of the steel plate. Therefore, the present disclosure limits an upper limit of the silicon (Si) content to 0.55%. A preferred upper limit of the silicon (Si) content may be 0.5%, and a more preferred upper limit of the silicon (Si) content may be 0.4%.

### Manganese (Mn): 0.9 to 1.75%

Manganese (Mn) may be an effective element for securing strength, and the present disclosure limits a lower limit of the manganese (Mn) content to 0.9% to achieve this effect. A preferred lower limit of the manganese (Mn) content may be 1.0%, and a more preferred lower limit of the manganese (Mn) content may be 1.2%. Manganese (Mn) may be combined with sulfur (S) to form a non-metallic inclusion such as MnS. When manganese (Mn) is added excessively, elongation at room temperature and low-temperature toughness may be deteriorated. Therefore, the present disclosure limits an upper limit of the manganese (Mn) content to 1.75%. A preferred upper limit of the manganese (Mn) content may be 1.7%, and a more preferred upper limit of the manganese (Mn) content may be 1.6%.

### Aluminum (Al): 0.001 to 0.05%

Since aluminum (Al) may be an element as a strong deoxidizer, the present disclosure limits a lower limit of the aluminum (Al) content to 0.001% for a deoxidation effect in a steelmaking process. When aluminum (Al) is added excessively, the deoxidation effect may be saturated, but manufacturing costs may be increased. The present disclosure limits an upper limit of the aluminum (Al) content to 0.05%. The aluminum (Al) content is more preferably 0.01 to 0.04%.

### Phosphorus (P): 0.03% or less

Phosphorus (P) may be an element that impairs low-temperature toughness. Therefore, P may be desirable to have its content managed to be as low as possible. Since Phosphorus (P) may be an element that may be inevitably contained in a steelmaking process, may take excessive cost to completely remove it, the present disclosure limits an upper limit of the phosphorus (P) content to 0.03%. A preferred upper limit of the phosphorus (P) content may be 0.02%, and a more preferred upper limit of the phosphorus (P) content may be 0.01%.

### Sulfur (S): 0.03% or less

Sulfur (S) may be also an element that adversely affects low-temperature toughness, together with phosphorus (P). Therefore, S may be desirable to have its content managed to be as low as possible. Since sulfur (S) may be an element that may be inevitably contained in a steelmaking process, like phosphorus (P), and may take excessive cost to completely remove it, the present disclosure limits an upper limit of the sulfur (S) content to 0.03%. A preferred upper limit of the sulfur (S) content may be 0.02%, and a more preferred upper limit of the sulfur (S) content may be 0.01%.

### Chromium (Cr): 0.05 to 0.3%

Since chromium (Cr) may be an element contributing to an increase in strength, the present disclosure limits a lower limit of the chromium (Cr) content to 0.05% to achieve this effect. Chromium (Cr) may be an expensive element. When Cr is added excessively, it is not preferable from a viewpoint of economic efficiency. Therefore, the present disclosure limits an upper limit of the chromium (Cr) content to 0.3%. Therefore, the chromium (Cr) content of the present disclosure may be 0.05 to 0.3%, and is more preferably 0.05 to 0.2%.

Nickel (Ni): 0.05 to 0.6%

Nickel (Ni) may be an effective element for improving low-temperature toughness. Therefore, the present disclosure limits a lower limit of the nickel (Ni) content to 0.05% to achieve this effect. Nickel (Ni) may be an expensive element. When Ni is excessively added, an increase in production cost may occur. Therefore, the present disclosure limits an upper limit of the nickel (Ni) content to 0.6%. Therefore, the nickel (Ni) content of the present disclosure may be 0.05 to 0.6%, and is more preferably 0.2 to 0.6%.

### Copper (Cu): 0.005 to 0.35%

Copper (Cu) may be an effective element for increasing strength. Therefore, the present disclosure limits a lower limit of the copper (Cu) content to 0.005% to achieve this effect. Copper (Cu) may be an expensive element. When Cu is excessively added, an increase in production cost may occur. Therefore, the present disclosure limits an upper limit of the copper (Cu) content to 0.35%. Therefore, the copper (Cu) content of the present disclosure may be 0.005 to 0.35%, and is more preferably 0.01 to 0.3%.

### Molybdenum (Mo): 0.05 to 0.2%

Molybdenum (Mo) may be an alloy element effective for improving strength, and may be an element that prevents crack generation caused by sulfide. Therefore, the present disclosure limits a lower limit of the molybdenum (Mo) content to 0.05% to achieve this effect. Molybdenum (Mo) may be also an expensive element. When Mo is excessively added, an increase in production cost may occur. Therefore, the present disclosure limits an upper limit of the molybdenum (Mo) content to 0.2%. Therefore, the molybdenum (Mo) content of the present disclosure is 0.05 to 0.2%, and is preferably 0.1 to 0.2%.

### Vanadium (V): 0.005 to 0.07%

Vanadium (V) may be an effective element for improving low-temperature toughness. Therefore, the present disclosure limits a lower limit of the vanadium (V) content to 0.005% to achieve this effect. Vanadium (V) may be also an expensive element. When V is excessively added, an increase in production cost may occur. Therefore, the present disclosure limits an upper limit of the vanadium (V) content to 0.07%. Therefore, the vanadium (V) content of the present disclosure is 0.005 to 0.07%, and is preferably 0.01 to 0.07%.

### Niobium (Nb): 0.005 to 0.04%

Niobium (Nb) may be an element that may be dissolved in austenite to increase hardenability of the austenite. In addition, niobium (Nb) may be an element that is precipitated as carbonitride (Nb (C,N)) matching with a matrix, together with titanium (Ti), and may be a major element for obtaining a tensile strength of 600 MPa or more for which the present disclosure seeks. Therefore, the present disclosure limits a lower limit of the niobium (Nb) content to 0.005% to achieve this effect. When niobium (Nb) is excessively added, coarse precipitates may occur in the process of continuous casting, and Nb may act as a starting point for hydrogen-induced cracking (HIC) . Therefore, the present disclosure limits an upper limit of the niobium (Nb) content to 0.04%. Therefore, the niobium (Nb) content of the present disclosure is 0.005 to 0.04%, and is preferably 0.01 to 0.03%.

### Calcium (Ca): 0.0005 to 0.005%

Calcium (Ca) may be combined with sulfur (S) to form a CaS precipitate, and may thus be an effective element for suppressing formation of MnS. Therefore, the present disclosure limits a lower limit of the calcium (Ca) content to 0.0005% to achieve this effect. When calcium (Ca) is excessively added, Ca may react with oxygen in steel to produce CaO, which may be a non-metallic inclusion. Therefore, the present disclosure limits an upper limit of the calcium (Ca) content to 0.005%. Therefore, the calcium (Ca) content of the present disclosure is 0.0005 to 0.005%, and is preferably 0.001 to 0.003%.

### Titanium (Ti): 0.005 to 0.025%

An appropriate content of titanium (Ti) may be fluidly limited according to the content of nitrogen (N). When the content of titanium (Ti) is relatively small, compared to the content of nitrogen (N), an amount of TiN produced may be relatively small, which may be disadvantageous for fine-graining. When titanium (Ti) is added in an excessive amount, TiN may become coarse during a heating operation to reduce an effect of inhibiting grain growth. Therefore, in consideration of the content (e.g., 0.002 to 0.006%) of nitrogen (N), the content of titanium (Ti) of the present disclosure is 0.005 to 0.025%, and is preferably 0.01 to 0.02%.

### Nitrogen (N): 0.002 to 0.006%

Nitrogen (N) may be widely known as an element that plays a role in increasing toughness of a base material and impact toughness of a heat-affected zone (HAZ) by forming a TiN precipitate with titanium (Ti) to refine grains. In this regard, according to the present disclosure, nitrogen (N) may be an element that should be added to achieve the purpose of grain refinement. Therefore, the present disclosure limits a lower limit of the nitrogen (N) content to 0.002% to achieve this effect. When the nitrogen (N) content is excessively added, an amount of TiN may be excessively increased and low-temperature toughness may be reduced. Therefore, the present disclosure limits an upper limit of the nitrogen (N) content to 0.006%. Therefore, the nitrogen (N) content of the present disclosure is 0.002 to 0.006%, and is preferably 0.002 to 0.004%.

### Boron (B): less than 0.0005%

In the present disclosure, the content of boron (B) may be actively suppressed, but excessive cost may be consumed to completely remove boron (B), which may be inevitably introduced during a steelmaking process. Therefore, the present disclosure limits the boron (B) content to less than 0.0005%. A preferred boron (B) content is 0.0002% or less, and a more preferred boron (B) content is 0.0001% or less.

A high strength steel plate according to an aspect of the present disclosure satisfies relationships of Cu + Ni + Cr + Mo: 1.5% or less, Cr + Mo: 0.4% or less, V + Nb: 0.1% or less, and Ca/S: 1.0 or higher.

Hereinafter, the relationships of the present disclosure will be described in more detail.
Cu + Ni + Cr + Mo: 1.5% or less
Cr + Mo: 0.4% or less
V + Nb: 0.1% or less
Ca/S: 1.0 or higher

The relationships of Cu + Ni + Cr + Mo, Cr + Mo, and V + Nb may be values that are respectively limited in the basic specification (ASTMA20) regarding steel for a pressure vessel, and the content of Cu + Ni + Cr + Mo is limited to 1.5% or less, the content of Cr + Mo is limited to 0.4% or less, and the content of V + Nb is limited to 0.1% or less. In addition, a ratio of Ca/s is an essential composition ratio of spheroidizing an MnS inclusion to improve hydrogen-induced crack resistance. When the ratio of Ca/s is less than 1.0, it may be difficult to expect the effect, the ratio is limited to satisfy 1.0 or more.

Hereinafter, the microstructure of the present disclosure will be described in more detail.

A high strength steel plate according to an aspect of the present disclosure includes a combined structure of tempered martensite and tempered bainite as a microstructure.

Microstructure: combined structure of tempered martensite and tempered bainite

When quenching and tempering a steel material provided with the above-described alloy composition, a microstructure of the steel material may have a microstructure of tempered martensite and tempered bainite. In the present disclosure, the tempered martensite and the tempered bainite includes 30 to 60 area% and 40 to 70 area%, respectively, and a tensile strength of 600 MPa, a nil-ductility transition temperature of -50°C or lower, and a Charpy impact toughness of 300 J or more at -60°C are effectively secured. A preferred area fraction of tempered martensite is 40 to 60%, and a preferred area fraction of tempered bainite is 40 to 60%. In addition, the sum of area fractions of the tempered martensite and the tempered bainite may be 100%.

Grain Aspect Ratio: 1.1 ≤ Long axis/Short axis ≤ 2.5

In the present disclosure, in order to secure high impact toughness and strength, a grain aspect ratio (a ratio of long axis/short axis) is controlled within a certain range, and the grain aspect ratio may be controlled by a rolling (a recrystallization control rolling) process. When the grain aspect ratio is less than 1.1, a shape of the grain may be rounded, surface energy thereof may become small, and it may be difficult to expect refinement of the grain. Therefore, it may be difficult to secure sufficient impact toughness and strength. In addition, when the grain aspect ratio exceeds 2.5, a rolling load for forming the grain becomes too high, and impact toughness may be lowered, which is not preferable. Therefore, the present disclosure limits the grain aspect ratio (the ratio of long axis/short axis) to have a range of 1.1 to 2.5.

Hereinafter, a manufacturing method of the present disclosure will be described in more detail.

A high strength steel plate according to an aspect of the present disclosure is manufactured by reheating a steel slab at 1050 to 1250°C, the steel slab including, by weight: 0.05 to 0.20% of C, 0.15 to 0.55% of Si, 0.9 to 1.75% of Mn, 0.001 to 0.05% of Al, 0.03% or less of P, 0.03% or less of S, 0.05 to 0.3% of Cr, 0.05 to 0.6% of Ni, 0.005 to 0.35% of Cu, 0.05 to 0.2% of Mo, 0.005 to 0.07% of V, 0.005 to 0.04% of Nb, 0.0005 to 0.005% of Ca, 0.005 to 0.025% of Ti, 0.002 to 0.006% of N, less than 0.0005% of B, and a balance of Fe, with inevitable impurities, satisfying relationships of Cu + Ni + Cr + Mo: 1.5% or less, Cr + Mo: 0.4% or less, V + Nb: 0.1% or less, and Ca/S: 1.0 or higher, rolling the slab in a temperature range of Tnr to Tnr + 100°C to provide a steel plate, austenizing the steel plate in a temperature range of 870 to 950°C, quenching the austenized steel plate to a temperature range of 300°C or lower, and tempering the quenched steel plate in a temperature range of 595 to 700°C.

Since an alloy composition and a content of the slab of the present disclosure correspond to the alloy composition and the content of the high strength steel plate described above, a description of the alloy composition and the content of the slab of the present disclosure may be replaced with the description of the alloy composition and the content of the steel plate described above.

Slab Reheating Operation: 1050 to 1250°C

In the present disclosure, a slab provided with the above-described alloy composition is reheated at a temperature range of 1050 to 1250°C. This is because, when a reheating temperature thereof is less than 1050°C, it may be difficult to sufficiently dissolve solute atoms, and when a reheating temperature thereof exceeds 1250°C, an austenite grain size may be excessively coarsened and properties of a steel plate may be deteriorated.

Recrystallization Control Rolling Operation: a temperature range of Tnr to (Tnr + 100°C), a cumulative reduction amount of 50 to 90% at a rolling reduction ratio of 10% or more per rolling pass

The recrystallization control rolling operation refers to a rolling operation to be performed at a temperature equal to or higher than an unrecrystallized temperature . In this case, the unrecrystallized temperature Tnr is derived by the following Equation 1, which has been already known. In the following Equation 1, a unit of each alloy element is weight%. $Tnr \left(°C\right) = 887 - 464 \times C + 890 \times Ti + 363 \times Al - 357 \times Si + \left(\begin{matrix}6445 \times Nb - 644 \times N \\ {b}^{1 / 2}\end{matrix}\right) + \left(732\times V-230\times {V}^{1 / 2}\right) .$

In order to improve strength, it may be necessary to refine an average particle diameter of prior austenite to 30 +µm or less in the recrystallization control rolling operation. When the average particle diameter of the prior austenite exceeds 30 µm, strength and toughness of a product may not be sufficiently exhibited. Therefore, a safety level high enough for a nuclear reactor containment vessel may not be guaranteed. To this end, in the present disclosure, the rolling operation is performed in a temperature range of Tnr to Tnr + 100°C.

In this case, a rolling reduction ratio of 10% or more may be applied per rolling pass, to finally perform the rolling operation in a cumulative reduction amount of 50 to 90%. Such a reduction amount is provided to control an average size (30 µm or less) of a microstructure required in the present disclosure and a grain aspect ratio (a long axis/short axis ratio) to 1.1 to 2.5. Therefore, when the cumulative reduction amount is less than 50%, it may be difficult to expect a refinement effect of the microstructure and a control effect of the grain aspect ratio. When the cumulative reduction amount exceeds 90%, a rolling load may be excessively applied, which may cause a problem in process.

Heat Treatment and Quenching Operation: quenching after austenizing the steel plate for a time period of 1.6 * t (where, t denotes a thickness (mm) of the steel plate) + (10 to 30 minutes) in a temperature range of 870 to 950°C

The quenching operation may be an important process for obtaining a combined structure of tempered martensite and tempered bainite, and may be necessary to strictly control process conditions to form a microstructure capable of securing a tensile strength of 600 MPa or more, a -60°C Charpy impact toughness of 300J or more, and a nil-ductility transition temperature property of -50°C or lower.

In the present disclosure, the austenizing operation may be performed for a time period of 1.6 * t (where, t denotes a thickness (mm) of the steel plate) + (10 to 30 minutes) in a temperature range of 870 to 950°C. The austenizing operation may be a heat treatment for austenizing the structure before the quenching operation. When a temperature range of the heat treatment is less than 870°C, it may be difficult to re-solidify the solute elements, and thus it may be difficult to secure strength. When a temperature range of the heat treatment exceeds 950°C, growth of grains may occur and coarse grains may occur, to impair low-temperature toughness. Therefore, a temperature range of the austenizing operation of the present disclosure may be limited to a temperature range of 870 to 950°C.

In addition, in the present disclosure, the austenizing operation may be performed for a time period of 1.6 * t (where, t denotes a thickness (mm) of the steel plate) + (10 to 30 minutes). When a time period of the austenizing operation is excessively short, an effect of sufficient austenizing may not be expected due to insufficient heating time, and it may be difficult to homogenize the structure. When a time period of the austenizing operation is excessively long, production time may be prolonged and productivity may be deteriorated. Therefore, a time period of the austenizing operation of the present disclosure may be limited to 1.6 * t (where, t denotes a thickness (mm) of the steel plate) + (10 to 30 minutes) . For reference, in the steel plate manufacturing process, when 1.6 * t is set as a heating time period, and a target temperature is reached, 10 to 30 minutes may be set as a maintenance time period to perform the austenizing operation.

The steel plate, after the austenizing operation, is quenched, preferably water-cooled, to be transformed to a combined structure of martensite and bainite. Conditions for the quenching operation in the present disclosure are not particularly limited, and any rapid quenching method including a water cooling operation may be applied to the quenching operation of the present disclosure. In order to obtain a microstructure desired by the present disclosure, after the austenizing operation is finished, the steel plate may be cooled to a temperature range of 300°C or lower.

Tempering Operation: 2.4 × t (where, t denotes a thickness (mm) of the steel plate) + (10 to 30 minutes) in a temperature range of 595 to 700°C

In the present disclosure, in order to secure excellent tensile strength, nil-ductility transition temperature, and low-temperature toughness properties, a tempering operation of the quenched steel material to 300°C or lower is used to remove residual stress in a structure thereof. Therefore, tempered martensite and tempered bainite is formed.

A temperature range of the tempering operation of the present disclosure is limited to 595 to 700°C. This is because, when a temperature range of the tempering operation is less than 595°C, carbides and the like may be not smoothly precipitated, and when a temperature range of the tempering operation exceeds 700°C, strength of the steel material may be lowered.

In addition, the tempering operation of the present disclosure may be carried out for a time period of 2.4 * t (where, t denotes a thickness (mm) of the steel plate) + (10 to 30 minutes) to obtain a sufficient tempering effect. For reference, in the steel plate manufacturing process, when 2.4 * t is set as a heating time period, and a target temperature is reached, 10 to 30 minutes may be set as a maintenance time period to perform the tempering operation.

### [Mode for Invention]

Hereinafter, the present disclosure will be described in more detail through examples. However, it may be necessary to note that the embodiments described below are only intended to further illustrate the present disclosure and are not intended to limit the scope of the present disclosure.

A slab provided with the alloy composition of Table 1 below was prepared.

**[Table 1]**

| Compositi on (wt%) | IS a | IS b | IS c | CS d | CS e | CS f |
|---|---|---|---|---|---|---|
| C | 0.10 | 0.09 | 0.12 | 0.06 | 0.07 | 0.09 |
| Mn | 1.51 | 1.58 | 0.92 | 1.30 | 1.35 | 0.78 |
| Al | 0.02 | 0.03 | 0.032 | 0.035 | 0.030 | 0.032 |
| Si | 0.35 | 0.36 | 0.36 | 0.35 | 0.34 | 0.36 |
| P | 0.009 | 0.010 | 0.008 | 0.008 | 0.010 | 0.010 |
| S | 0.0010 | 0.0008 | 0.0011 | 0.0013 | 0.0014 | 0.0012 |
| Cu | 0.03 | 0.04 | 0.03 | 0.05 | - | - |
| Ni | 0.50 | 0.55 | 0.53 | 0.05 | 0.15 | 0.10 |
| Cr | 0.05 | 0.05 | 0.06 | 0.03 | 0.05 | 0.04 |
| Mo | 0.15 | 0.18 | 0.17 | 0.15 | 0.10 | 0.16 |
| V | 0.030 | 0.025 | 0.030 | 0.003 | 0.005 | 0.030 |
| Nb | 0.012 | 0.014 | 0.013 | 0.013 | 0.012 | 0.015 |
| B | - | - | - | 0.0015 | 0.0012 | 0.0007 |
| Ti | 0.012 | 0.010 | 0.013 | 0.013 | 0.012 | 0.013 |
| N | 0.0028 | 0.0035 | 0.0034 | 0.0028 | 0.0035 | 0.0032 |
| Ca | 0.0020 | 0.0019 | 0.0021 | 0.0018 | 0.0021 | 0.0020 |

| | | | | | | |
|---|---|---|---|---|---|---|
| IS: Inventive Steel, CS: Comparative Steel | | | | | | |

Test pieces were prepared by performing a reheating operation, a recrystallization control rolling operation, an austenizing operation, a quenching operation, and a tempering operation using respective slabs made of the compositions of Inventive Steel and Comparative Steel, as illustrated in Table 2 below. Properties such as strength, low-temperature toughness, and nil-ductility transition temperature were evaluated, and the results therefrom are illustrated in Table 3 below. In Table 3 below, the low-temperature impact toughness may be evaluated as a Charpy impact energy value obtained by performing a Charpy impact test on a specimen having a V notch at -60°C. In addition, the nil-ductility transition temperature may be a result value according to the drop-weight test transition temperature set by the ASTM E208-06 method.

**[Table 2]**

| | Condition | Steel Plate Thickness (mm) | Slab Reheatin g Temp. (°C) | Rolling Temp. (°C) | Recrystallization Control Rolling Cumulative Reduction Amount (%) | Grain Aspect Ratio* | Austenizing Temp. (°C) | Tempering Temp. (°C) |
|---|---|---|---|---|---|---|---|---|
| IS a | a-1 | 45 | 1200 | 780 | 60 | 1.75 | 900 | 680 |
| | a-2 | 80 | 1180 | 780 | 55 | 1.95 | 920 | 660 |
| | a-3 | 100 | 1100 | 790 | 50 | 1.25 | 910 | 650 |
| | a-4 | 50 | 1100 | 790 | 45 | 1.01 | 910 | 660 |
| IS b | b-1 | 45 | 1150 | 780 | 70 | 2.15 | 910 | 680 |
| | b-2 | 80 | 1100 | 780 | 60 | 2.00 | 920 | 660 |
| | b-3 | 100 | 1100 | 790 | 55 | 1.65 | 900 | 650 |
| IS c | C | 50 | 1150 | 780 | 75 | 1.98 | 900 | 660 |
| CS d | d-1 | 45 | 1200 | 780 | 20 | 1.02 | 920** | 680 |
| | d-2 | 100 | 1150 | 790 | 30 | 1.05 | 900** | 650 |
| CS e | E | 100 | 1100 | 780 | 40 | 1.06 | 900** | 650 |
| CS f | f | 80 | 1150 | 790 | 55 | 1.03 | 900 | 650 |

| | | | | | | | | |
|---|---|---|---|---|---|---|---|---|
| IS: Inventive Steel, CS: Comparative Steel * Grain aspect ratio: Long grain/short grain ** Quenching temperatures of Comparative Steel are normalizing temperatures | | | | | | | | |

**[Table 3]**

| | Condit ion | Tempered Martensite Structural Fraction (%) | Tempered Bainite Structural Fraction (%) | YS (MPa) | TS (MPa) | -60°C Impact Toughne ss (J)*** | NDT Transition Temp. (°C)**** | |
|---|---|---|---|---|---|---|---|---|
| IS a | a-1 | 56 | 44 | 634 | 649 | 334 | -80 | IE 1 |
| | a-2 | 51 | 49 | 641 | 641 | 324 | -70 | IE 2 |
| | a-3 | 48 | 52 | 628 | 634 | 313 | -65 | IE 3 |
| | a-4 | 62 | 38 | 580 | 701 | 58 | -40 | CE 1 |
| IS b | b-1 | 58 | 42 | 642 | 660 | 324 | -85 | IE 4 |
| | b-2 | 50 | 50 | 648 | 652 | 318 | -70 | IE 5 |
| | b-3 | 45 | 55 | 634 | 635 | 334 | -70 | IE 6 |
| IS c | C | 55 | 45 | 542 | 650 | 320 | -80 | IE 7 |
| CS d | d-1 | 85 | 15 | 370 | 639 | 180 | -40 | CE 2 |
| | d-2 | 80 | 20 | 365 | 630 | 172 | -45 | CE 3 |
| CS e | E | 82 | 18 | 358 | 630 | 193 | -40 | CE 4 |
| CS f | F | 85 | 15 | 443 | 650 | 140 | -30 | CE 5 |

| | | | | | | | | |
|---|---|---|---|---|---|---|---|---|
| IE: Inventive Example, CE: Comparative Example, IS: Inventive Steel, CS: Comparative Steel *** Impact toughness: impact toughness in a T direction (having a V-notch in a direction, perpendicular to a rolling direction) **** NDT transition temperature: transition temperature of the drop-weight test conducted by the ASTM208-06 method. | | | | | | | | |

As in the results of Tables 2 and 3, it can be seen that Inventive Examples 1 to 7 have microstructures of 30 to 60% of tempered martensite and 40 to 70% of tempered bainite, and secure a tensile strength of 600 MPa or more, an impact toughness of 300 J or more at -60°C, and a nil-ductility transition temperature property of -50°C or lower.

In a case of Comparative Example 1, it can be seen that, since a steel composition satisfies the defined steel composition of the present disclosure, but a cumulative reduction amount of a recrystallization control rolling operation does not satisfy the defined scope of the present disclosure, the area fractions of a microstructure defined by the present disclosure are not satisfied, and a nil-ductility transition temperature property at -50°C or lower is, thus, not secured.

In addition, in cases of Comparative Examples 2 to 5, it can be seen that, since steel compositions do not satisfy the defined steel composition of the present disclosure, a microstructure has 80 area% or more of tempered martensite and 20 area% or less of tempered bainite, and tensile strength, impact toughness, and nil-ductility transition temperature properties are degraded.

Therefore, since a steel plate according to an embodiment of the present disclosure may control a steel composition, a microstructure, and manufacturing operations under optimal conditions, to secure tensile strength of 600 MPa or more, Charpy impact toughness of 300 J or more at -60°C, and a nil-ductility transition temperature of -50°C or lower, a high strength steel plate having properties suitable for a nuclear reactor containment vessel may be provided.

While example embodiments have been illustrated and described above, it will be apparent to those skilled in the art that modifications and variations could be made without departing from the scope of the present disclosure as defined by the appended claims.

## Claims

1. A high strength steel plate comprising, by weight: 0.05 to 0.20% of C, 0.15 to 0.55% of Si, 0.9 to 1.75% of Mn, 0.001 to 0.05% of Al, 0.03% or less of P, 0.03% or less of S, 0.05 to 0.3% of Cr, 0.05 to 0.6% of Ni, 0.005 to 0.35% of Cu, 0.05 to 0.2% of Mo, 0.005 to 0.07% of V, 0.005 to 0.04% of Nb, 0.0005 to 0.005% of Ca, 0.005 to 0.025% of Ti, 0.002 to 0.006% of N, less than 0.0005% of B, and a balance of Fe, with inevitable impurities, satisfying relationships of Cu + Ni + Cr + Mo: 1.5% or less, Cr + Mo: 0.4% or less, V + Nb: 0.1% or less, and Ca/S: 1.0 or higher, and comprising a microstructure of 30 to 60 area% of tempered martensite and 40 to 70 area% of tempered bainite, wherein the sum of the tempered martensite and the tempered bainite is 100 area%, wherein a grain aspect ratio as defined herein of the microstructure is 1.1 to 2.5,
wherein Charpy impact toughness of the steel plate is 300J or more at -60°C, and wherein the low-temperature impact toughness is evaluated as a Charpy impact energy value obtained by performing a Charpy impact test on a specimen having a V notch at -60°C **,** and wherein the tensile strength of the steel plate is 600 MPa or more.

2. The high strength steel plate according to claim 1, wherein the tempered martensite comprises 40 to 60 area% in the microstructure, and the tempered bainite comprises 40 to 60 area% in the microstructure.

3. The high strength steel plate according to any one of claims 1 to 3, wherein a nil-ductility transition temperature of the steel plate is -50°C or lower and wherein the nil-ductility transition temperature is a result value according to the drop-weight test transition temperature set by the ASTM E208-06 method.

4. A method of manufacturing a high strength steel plate, comprising:
reheating a steel slab at 1050 to 1250°C, the steel slab comprising, by weight: 0.05 to 0.20% of C, 0.15 to 0.55% of Si, 0.9 to 1.75% of Mn, 0.001 to 0.05% of Al, 0.03% or less of P, 0.03% or less of S, 0.05 to 0.3% of Cr, 0.05 to 0.6% of Ni, 0.005 to 0.35% of Cu, 0.05 to 0.2% of Mo, 0.005 to 0.07% of V, 0.005 to 0.04% of Nb, 0.0005 to 0.005% of Ca, 0.005 to 0.025% of Ti, 0.002 to 0.006% of N, less than 0.0005% of B, and a balance of Fe, with inevitable impurities, satisfying relationships of Cu + Ni + Cr + Mo: 1.5% or less, Cr + Mo: 0.4% or less, V + Nb: 0.1% or less, and Ca/S: 1.0 or higher,
rolling the slab in a temperature range of Tnr to Tnr + 100°C, wherein Tnr is determined in accordance with Equation 1 hereof and a unit of each alloy element is weight%, to provide a steel plate,
austenizing the steel plate in a temperature range of 870 to 950°C,
quenching the austenized steel plate to a temperature range of 300°C or lower, and tempering the quenched steel plate in a temperature range of 595 to 700°C, wherein a cumulative reduction amount of the rolling is 50 to 90%, and wherein a grain aspect ratio as defined herein of a microstructure of the steel plate by the rolling is controlled to have a range of 1.1 to 2.5, $Tnr \left(°C\right) = 887 - 464 \times C + 890 \times Ti + 363 \times Al - 357 \times Si + \left(\begin{matrix}6445 \times Nb - 644 \times N \\ {b}^{1 / 2}\end{matrix}\right) + \left(732\times V-230\times {V}^{1 / 2}\right) .$

5. The method according to claim 4, wherein the austenizing is performed for a time period of 1.6 * t +(10 to 30 minutes) wherein t denotes a thickness in mm of the steel plate.

6. The method according to claim 4, wherein the tempering is performed for a time period of 2.4 * t + (10 to 30 minutes) , wherein t denotes a thickness in mm of the steel plate.

## Patentansprüche

1. Hochfestigkeitsstahlplatte, die nach Gewicht Folgendes umfasst: 0,05 bis 0,20 % C, 0,15 bis 0,55 % Si, 0,9 bis 1,75 % Mn, 0,001 bis 0,05 % Al, 0,03 % oder weniger P, 0,03 % oder weniger S, 0,05 bis 0,3 % Cr, 0,05 bis 0,6 % Ni, 0,005 bis 0,35 % Cu, 0,05 bis 0,2 % Mo, 0,005 bis 0,07 % V, 0,005 bis 0,04 % Nb, 0,0005 bis 0,005 % Ca, 0,005 bis 0,025 % Ti, 0,002 bis 0,006 % N, weniger als 0,0005 % B und einen Rest an Fe mit unvermeidlichen Verunreinigungen, die die Beziehungen Cu + Ni + Cr + Mo: 1,5 % oder weniger, Cr+ Mo: 0,4 % oder weniger, V + Nb: 0,1 % oder weniger und Ca/S: 1,0 oder höher erfüllt und eine Mikrostruktur von 30 bis 60 Flächen-% von angelassenem Martensit und 40 bis 70 Flächen-% von angelassenem Bainit umfasst, wobei die Summe des angelassenen Martensits und des angelassenen Bainits 100 Flächen-% beträgt, wobei, wie hierin definiert, ein Partikelseitenverhältnis der Mikrostruktur 1,1 bis 2,5 beträgt,
wobei die Charpy-Schlagzähigkeit der Stahlplatte 300 J oder mehr bei -60 °C beträgt und wobei die Niedrigtemperaturschlagzähigkeit als ein Charpy-Schlagzähigkeitsenergiewert bewertet wird, der durch Durchführen eines Charpy-Schlagtests an einer Probe, die eine V-Kerbe bei -60 °C aufweist, erhalten wird und wobei die Zugfestigkeit der Stahlplatte 600 MPa oder mehr beträgt.

2. Hochfestigkeitsstahlplatte nach Anspruch 1, wobei der angelassene Martensit 40 bis 60 Flächen-% in der Mikrostruktur umfasst und der angelassene Bainit 40 bis 60 Flächen-% in der Mikrostruktur umfasst.

3. Hochfestigkeitsstahlplatte nach einem der Ansprüche 1 bis 3, wobei eine Nullduktilitätsübergangstemperatur der Stahlplatte -50 °C oder niedriger beträgt und wobei die Nullduktilitätsübergangstemperatur ein Ergebniswert gemäß der Fallgewichtstestübergangstemperatur ist, die durch das ASTM E208-06 Verfahren eingestellt wird.

4. Verfahren zum Herstellen einer Hochfestigkeitsstahlplatte, das Folgendes umfasst:
Wiedererwärmen einer Stahlbramme bei 1050 bis 1250 °C, wobei die Stahlbramme nach Gewicht Folgendes umfasst: 0,05 bis 0,20 % C, 0,15 bis 0,55 % Si, 0,9 bis 1,75 % Mn, 0,001 bis 0,05 % Al, 0,03 % oder weniger P, 0,03 % oder weniger S, 0,05 bis 0,3 % Cr, 0,05 bis 0,6 % Ni, 0,005 bis 0,35 % Cu, 0,05 bis 0,2 % Mo, 0,005 bis 0,07 % V, 0,005 bis 0,04 % Nb, 0,0005 bis 0,005 % Ca, 0,005 bis 0,025 % Ti, 0,002 bis 0,006 % N, weniger als 0,0005 % B und einen Rest an Fe mit unvermeidlichen Verunreinigungen, die die Beziehungen Cu + Ni + Cr + Mo: 1,5 % oder weniger, Cr + Mo: 0,4 % oder weniger, V + Nb: 0,1 % oder weniger und Ca/S: 1,0 oder höher erfüllt,
Walzen der Bramme in einem Temperaturbereich von Tnr bis Tnr + 100 °C, wobei Tnr gemäß Gleichung 1 hiervon bestimmt wird und eine Einheit jedes Legierungselements Gewichtsprozent ist, um eine Stahlplatte bereitzustellen,
Austenitisieren der Stahlplatte in einem Temperaturbereich von 870 bis 950 °C,
Abschrecken der austenitisierten Stahlplatte auf einen Temperaturbereich von 300 °C oder niedriger und
Anlassen der abgeschreckten Stahlplatte in einem Temperaturbereich von 595 bis 700 °C, wobei eine kumulative Reduktionsmenge des Walzens 50 bis 90 % beträgt und wobei, wie hierin definiert, ein Partikelseitenverhältnis einer Mikrostruktur der Stahlplatte durch das Walzen gesteuert wird, um einen Bereich von 1,1 bis 2,5 aufzuweisen, $Tnr \left(°C\right) = 887 - 464 \times C + 890 \times Ti + 363 \times Al - 357 \times Si + \left(6445\times Nb-644\times N {b}^{1 / 2}\right) + \left(\begin{matrix}732 \times V - \\ 230 \times {V}^{1 / 2}\end{matrix}\right) .$

5. Verfahren nach Anspruch 4, wobei das Austenitisieren eine Zeitdauer von 1,6 * t + (10 bis 30 Minuten) lang durchgeführt wird, wobei t eine Dicke in mm der Stahlplatte bezeichnet.

6. Verfahren nach Anspruch 4, wobei das Anlassen eine Zeitdauer von 2,4 * t + (10 bis 30 Minuten) lang durchgeführt wird, wobei t eine Dicke in mm der Stahlplatte bezeichnet.

## Revendications

1. Tôle d'acier à haute résistance comprenant, en poids : 0,05 à 0,20 % de C, 0,15 à 0,55 % de Si, 0,9 à 1,75 % de Mn, 0,001 à 0,05 % d'Al, 0,03 % ou moins de P, 0,03 % ou moins de S, 0,05 à 0,3 % de Cr, 0,05 à 0,6 % de Ni, 0,005 à 0,35 % de Cu, 0,05 à 0,2 % de Mo, 0,005 à 0,07 % de V, 0,005 à 0,04 % de Nb, 0,0005 à 0,005 % de Ca, 0,005 à 0,025 % de Ti, 0,002 à 0,006 % de N, moins de 0,0005 % de B, et un complément de Fe, avec des impuretés inévitables, satisfaisant les relations Cu + Ni + Cr + Mo : 1,5 % ou moins, Cr + Mo : 0,4 % ou moins, V + Nb : 0,1 % ou moins, et Ca/S : 1,0 ou plus, et comprenant une microstructure de 30 à 60 % en surface de martensite revenue et de 40 à 70 % en surface de bainite revenue, la somme de la martensite revenue et de la bainite revenue étant de 100 % en surface, un rapport d'aspect des grains tel que défini ici de la microstructure étant de 1,1 à 2,5, la résistance au choc Charpy de la tôle d'acier étant de 300 J ou plus à -60 °C, et la résistance au choc à basse température étant évaluée en tant que valeur d'énergie de choc Charpy obtenue en effectuant un essai de choc Charpy sur un échantillon ayant une entaille en V à -60 °C, et la résistance à la traction de la tôle d'acier étant de 600 MPa ou plus.

2. Tôle d'acier à haute résistance selon la revendication 1, dans laquelle la martensite revenue comprend 40 à 60 % en surface dans la microstructure, et la bainite revenue comprend 40 à 60 % en surface dans la microstructure.

3. Tôle d'acier à haute résistance selon l'une quelconque des revendications 1 à 3, dans laquelle une température de ductilité nulle de transition de la tôle d'acier est de -50 °C ou moins et dans laquelle la température de ductilité nulle de transition est une valeur de résultat selon la température de transition d'essai au mouton fixée par le procédé ASTM E208-06.

4. Procédé de fabrication d'une tôle d'acier à haute résistance, comprenant :
le réchauffage d'une brame d'acier de 1 050 à 1 250 °C, la brame d'acier comprenant en poids : 0,05 à 0,20 % de C, 0,15 à 0,55 % de Si, 0,9 à 1,75 % de Mn, 0,001 à 0,05 % d'Al, 0,03 % ou moins de P, 0,03 % ou moins de S, 0,05 à 0,3 % de Cr, 0,05 à 0,6 % de Ni, 0,005 à 0,35 % de Cu, 0,05 à 0,2 % de Mo, 0,005 à 0,07 % de V, 0,005 à 0,04 % de Nb, 0,0005 à 0,005 % de Ca, 0,005 à 0,025 % de Ti, 0,002 à 0,006 % de N, moins de 0,0005 % de B, et un complément de Fe, avec des impuretés inévitables, satisfaisant les relations Cu + Ni + Cr + Mo : 1,5 % ou moins, Cr + Mo : 0,4 % ou moins, V + Nb : 0,1 % ou moins, et Ca/S : 1,0 ou plus,
le laminage de la brame dans une plage de températures de Tnr à Tnr + 100 °C, Tnr étant déterminé conformément à l'équation 1 de la présente et une unité de chaque élément d'alliage étant un % en poids, pour fournir une tôle d'acier,
l'austénisation de la tôle d'acier dans une plage de température de 870 à 950 °C,
la trempe de la tôle d'acier austénisée jusqu'à une plage de températures de 300 °C ou moins, et
le revenu de la tôle d'acier trempée dans une plage de températures de 595 à 700 °C, une quantité de réduction cumulative du laminage étant de 50 à 90 %, et un rapport d'aspect de grain tel que défini ici d'une microstructure de la tôle d'acier par le laminage étant régulé pour avoir une plage de 1,1 à 2,5, $Tnr \left(°C\right) = 887 - 464 \times C + 890 \times Ti + 363 \times Al - 357 \times Si + \left(\begin{matrix}6445 \times Nb - \\ 644 \times {Nb}^{1 / 2}\end{matrix}\right) + \left(732\times V-230\times {V}^{1 / 2}\right) .$

5. Procédé selon la revendication 4, dans lequel l'austénisation est effectuée pendant une période de 1,6 * t + (10 à 30 minutes), t désignant une épaisseur en mm de la tôle d'acier.

6. Procédé selon la revendication 4, dans lequel le revenu est effectué pendant une période de 2,4 * t + (10 à 30 minutes), t désignant une épaisseur en mm de la tôle d'acier.
